

## UNITED STATES PATENT OFFICE

2,233,203

## LUBRICATING OIL

Marcellus T. Flaxman, Wilmington, Calif., assignor to Union Oil Company of California, Los Angeles, Calif., a corporation of California

No Drawing. Application May 3, 1938,  
Serial No. 205,725

16 Claims. (Cl. 252—39)

This invention relates to lubricating oils and particularly to mineral lubricating oils adapted for use in severe service internal combustion engines such as Diesel engines and high output 5 aviation engines.

The object of the invention is to provide mineral lubricating oils which will be highly stable against deterioration in use and will largely overcome the sticking of piston rings, valves and the like and the formation of sludges or sludge or lacquer deposits on engine parts and will be free from corrosive influences upon crank shaft bearings, wrist pin bushings and other parts of the mentioned types of internal combustion engines.

Compositions suitable for these purposes belong to the class of compounds which are referred to as oil-soluble soaps. These oil-soluble soaps exhibit a permanent state of solubility or dispersion in the lubricating oil as distinguished 20 from soaps which tend to cloud or gel or stratify in the oil, at least in the proportions in which they are used for the present purposes.

## STATEMENT OF INVENTION

Primarily, the present invention resides in the employment in appropriate mineral lubricating oils of oil-soluble or dispersible metal soaps, such as alkaline earth metal soaps, or other suitable oil-soluble or dispersible soaps, of acids which 30 will be referred to here as pine acids or rosin acids or abietic acids. These soaps are to be added to suitable mineral lubricating oils (preferably naphthenic base oils) hereinafter described in small proportions insufficient to impart 35 a grease-like consistency, and preferably within limits of about 0.5% to 2.5% or 3%, or between about 1% and 2%, e. g. around 1.5%. The invention also resides in the use additionally of herein indicated types of soaps of what may 40 be referred to as pine fatty acids, or soap of other suitable high molecular weight fatty acids, and the invention further resides in the use of all these various soaps where they are also chlorinated or sulfurized or sulfo-chlorinated. 45 The use of chlorine and sulfur is to impart certain oiliness and extreme pressure characteristics which are desirable.

To obtain the advantages of sulfur, it is also desirable to employ a naphthenic base mineral 50 lubricating oil naturally containing sulfur sufficient to meet the requirements, for example from about one-half percent sulfur to 4% or 5% sulfur. The use of such sulfur-bearing oils is valuable to offset corrosive conditions which 55 are imparted where chlorine is present and especially to offset tendencies toward corrosion by organic acids of highly corrosion-sensitive alloy bearings, for example cadmium silver bearings, where the soaps tend to hydrolyze and promote 60 corrosive conditions. The invention therefore

resides also in the employment of pine acid or rosin acid soaps of the indicated types in mineral lubricating oils containing appreciable sulfur content as indicated, either naturally or by sulfurization of the soaps themselves. About 1% to about 3% combined sulfur such as naturally-occurring sulfur represents ordinarily a preferable range. 5

The invention also resides in such soap-containing oils wherein a small acid number exists, such as 0.2 to 0.5 as hereinafter indicated, whereby oil-solubility is improved and gelation in presence of small water content is avoided. 10

## DEFINITIONS

15

Where the term "rosin acids" or "pine acids" is used, I mean primarily abietic acid which ordinarily predominates in rosin and rosin oil and in oils which are marketed as "tallol" or "tall oil," and may be present in other resins. 20 While these materials include kindred acids such as d-pimamic acid and sapinic acids, and apparently also various isomers and polymers of these acids, the term "abietic acid" in general is intended to include also the mentioned variations. The term "pine acids" or "rosin acids" likewise is intended to signify the various abietic and kindred acidic materials and other saponifiable materials found in rosin, rosin oil, tall oil and the like. Apparently all of these materials are 25 valuable for the purposes here stated, and it is therefore possible, and within the scope of this invention, to produce soaps from the separated abietic acids or other indicated kindred acids or esters or from the rosin or rosin oil or tall oil themselves, and these materials are intended 30 to be included in terms such as "rosin acids" and "pine acids". 35

For the purposes of this disclosure abietic acid (C<sub>19</sub>H<sub>28</sub>COOH) is assumed to have the following 40 probable structural formula which is commonly accepted by many investigators as being representative of what is commonly known as abietic acid:



This formula may or may not actually indicate the true structure but it is presented as indicative of present chemical knowledge on the sub- 60

ject and for the purpose of making as full and clear a disclosure as possible.

With further reference to the terms "rosin acids" and "abietic acids," it is intended to include all those rosin materials which contain acids akin to abietic acid and produce the desired soaps of the present invention. As is well known, rosin is the relatively high melting point residue obtained from the distillation of natural crude turpentine from living trees and known as "gum rosin," or from the steam distillation or solvent extraction of the wood of pines and firs, such as cured or "fatty" pine stumps, and known as "wood rosin." The turpentine passes off under low temperature distillation conditions to form "gum turpentine" when the exudate from the living tree is distilled, and to form "wood turpentine" when the products from old or cured wood are distilled. From these rosin residues left after the turpentine has been distilled off, normally liquid rosin oils may be distilled out in one or more fractions including redistillation if desired, leaving a still higher melting point gum or wood rosin as the case may be.

The materials from wood distillation correspond generally with those from the living trees but differ in some particulars not clearly understood. However all of these rosin oils and rosins contain abietic acids and may be used for the present purposes. Apparently the abietic acids which are distilled over in the rosin oils are of lower molecular weight than the polymers remaining in the rosin bottoms; or the different abietic acids may be isomers of one another. The constitution above given for abietic acids is furnished as merely representative and there are undoubtedly many so-called abietic acids of varying constructions.

It is generally understood that abietic acid as such does not exist in the natural secretions and that other constituents, possibly isomers, are present having about the same composition as abietic acid itself, namely  $C_{19}H_{28}COOH$ . In any event, heat treatment and also acid treatment yield abietic acid, and it would appear that heavier heat treatment yields various isomers of abietic acid and probably polymers thereof also. These acids, which are commonly referred to as abietic acid and are here generally considered as consisting of abietic acid and its polymers principally but containing also d-pimamic and sapinic acids, are in general the acids intended when the term "rosin acids" is employed, this term including also the various isomers and polymers of these acids and kindred acids present in or obtainable from rosin.

With respect to the commercial product known as "tall oil," this is said to be defined as a waste material or by-product which is recovered from the wood of coniferous trees during the process of conversion of the wood fibre into cellulose by the so-called sulfate or Swedish process for cellulose pulp making. The residual waste liquor obtained from the process after the separation of the cellulose therefrom separates into two layers, the top layer of which is skimmed off and represents the crude tall oil. It is an oil of a strong tarry odor before purification and has chemical properties between those of fatty acids and those of resinic acids due to the fact that the tall oil always contains both fatty acids and resinic acids as two constituents. If desired, the tall oil may be purified by distillation or by any other known or preferred process. Either the purified

or the crude tall oil may be employed in the compounds of the present invention.

The percentages of fatty acids in tall oil vary from about 20% to about 50% or 60%, and the rosin acids vary from about 70% to about 20%, the remainder being sterols, other higher alcohols and hydrocarbons apparently. The fatty acids apparently are characteristic pine acids and not necessarily those commonly implied in the term "fatty acids," and may be designated by the term "pine fatty acids." This fatty acid content is largely unsaturated as indicated by the iodine number, the unsaturation apparently being of the oleic acid type. Presumably these unsaturated acids correspond largely with oleic acid or the closely related acids such as linoleic and linolenic, and possibly also in minor proportions with such higher acids as myristoleic and palmitoleic and heavier acids such as the elaeostearic, and erucic acids. However, since oleic acid is known generally to predominate in nature, these pine fatty acids as a whole are herein generally considered from the standpoint of oleic acid constitution.

25

#### OPERATING PROCEDURES

The preparation of soaps of abietic acid or rosin acids will be considered from the standpoint of calcium soaps made by the saponification of rosin, or rosin purified to increase the abietic acid content, or rosin oil, which will in general be also applicable to the preparation of such soaps from tall oil or purified or partially purified or segregated rosin acids such as commercial abietic acid, where available. In the saponification of rosin to produce calcium soaps thereof, or in the saponification of rosin oils or the like, the rosin or rosin oils preferably will be dissolved at suitably elevated temperature, for example 250° F. in the case of rosin, in an appreciable quantity of the mineral lubricating oil to be used in preparing the final product. For example 1 to 10 volumes of lubricating oil based on the rosin may be employed. To this oil solution of rosin or rosin oil will be introduced preferably an excess of hydrated lime, (about 15% to 20% based on the rosin or rosin oil) and if desired a small quantity of water such as one-tenth of 1% of the total. This mixture will then be raised to a temperature of about 275° F. or in the range of 250° F. to 350° F. and maintained for a period of about two to five hours to effect neutralization of the rosin acids to the desired extent. This neutralization may be complete if desired or it may be such as to leave any desired or appropriate acid number. In employing 1 or 2 volumes of oil to 1 volume of rosin or rosin oil, the resultant mass will be more in the nature of a grease and this mass may then be diluted with more mineral oil to yield a suitable oil-soap concentrate of any desired soap content such as from 5% to 40% soap.

On the other hand, the total amount of oil desired in the concentrate may be added before saponification is undertaken and the entire mass subjected to the above indicated temperature range to obtain the desired extent of neutralization. Ordinarily the time for saponification will be greater than with the smaller amount of mineral oil. After the desired degree of neutralization has been effected, the mass will be brought to a temperature of around 325° F. to 350° F. to insure easy filtration or separation of solids and

50

55

60

65

70

75

75

## Soaps

also to accomplish sufficient dehydration to insure against any subsequent tendency to gel. For the purpose of removing solids centrifuging may be employed, or a small quantity of diatomaceous earth or other suitable filter aid will be supplied to the oil-soap mass to insure better removal of excess lime and the hot mass then filtered through a filter precoated with a small quantity of diatomaceous earth or other appropriate filter aid. In the use of filter aids care should be taken to avoid the use of those of a character or in quantity sufficient to effect substantial removal of the soaps from the oil as by adsorption. These filtrates when cooled constitute oil-soap concentrates which may be subsequently employed for addition to further amounts of the selected mineral lubricating oil stock in preparing final blends containing the indicated desired amounts of soaps, for example around 1% to 2% or more, particularly in the order of about 1.5%.

## Water and acid contents

With reference to dehydration and neutralization, the degree of dehydration should preferably be such that any tendency of the oil-soap mixtures to gel will be overcome. As a general guide, it may be said that in the case of concentrates containing about 40% rosin acid soaps or saponified products above described, the water content preferably should be well under 1%, and for concentrations around 8% or 10%, the water content should be less than about one-fourth of 1%, and in a final blend containing about 1.25% to 1.5% of soap, the water content should be under 0.1% or preferably under about 0.05%.

However, it has been found that by effecting an acid number in the soap corresponding to an acid number in the final blend of about 0.2 to 0.3 or in some cases 0.4 or 0.5, the water tolerance of the blends is increased. For example a blend having an acid number of .36 was highly resistant or tolerant toward the presence of 0.1% to 0.2% water without gelation. Also, another function of such free acid is to insure retention of the soaps in the oils. An acid number of 0.35 to 0.5 insures against the substantial formation of heavy bodied or viscous emulsions with the larger amounts of moisture.

By acid number is meant the amount of KOH in milligrams necessary to neutralize the acidity in one gram of the compounded product, and refers to the A. S. T. M. Method B for "Compounded Petroleum Products" as distinguished from Method A for "Petroleum Products." These methods are found in the A. S. T. M. Standards for 1936 test number D188-27T described on pages 629 to 631. It is to be understood that the acid numbers here given relate to final blends containing about 1.5% calcium rosin acid soaps calculated as calcium abietate or kindred soaps produced from rosins or rosin oils and the like.

In neutralizing rosin or rosin oil or rosin acids or tall oil, the desired acid number may be obtained by limiting the quantity of hydrated lime employed, or by limiting the heating time to effect only the desired degree of neutralization, or more conveniently by adding to a neutral concentrate prepared with an excess of lime a suitably calculated quantity of rosin or rosin oil or commercial abietic acid or other material containing the desired abietic acid. The acid number in the concentrate is of course adjusted so as to yield the desired acid number in the final blend above indicated.

In the use of tall oil, similar procedures are followed in the preparation of the soaps, but the resultant soaps, instead of being largely rosin acid soaps as is the case where rosin and rosin oils are employed, will be a mixture of rosin acid soaps and fatty acid soaps by reason of the fact that tall oil, as heretofore outlined, contains not only rosin acids, particularly abietic acid but also fatty acids obtained from the coniferous wood employed. Since tall oil varies in content of fatty acids ("pine fatty acids") and rosin acids, as previously indicated, the mixed soaps will vary accordingly. There are certain advantages in the use of these mixed soaps in that they act as common solvents for each other and the fatty acid soaps appear to serve to stabilize the rosin acid soaps and retain them in the lubricating oil. In the use of these mixed soaps the total soap is considered in calculating the soap content in the concentrate or final blend. In some cases, the commonly known fatty acids may also be employed with the rosin acids or abietic acids herein described when preparing soaps of this invention.

In the preparation of soaps of the acidic materials herein described, the calcium soaps are preferred insofar as present developments are concerned because they are adequately oil-soluble under the conditions described and are more or less conveniently prepared. Likewise they are highly efficient for the purposes described. On the other hand, the invention is not limited to the use of calcium soaps but may employ in some cases other soaps particularly soaps of aluminum, magnesium and zinc. Also it is possible to use soaps of sodium, potassium, tin, manganese and the like for certain purposes and likewise soaps of organic bases such as amyl amine, cyclo hexyl amine, morpholine, triethanolamine and the like. It is to be understood, however, that none of these soaps are now considered to be the full equivalents of calcium soap. In some instances these various other soaps may be used in various combinations with each other and with the preferred calcium soaps; for example triethanolamine soap may be used with the calcium soap.

As a possible source of abietic acid or other rosin acids in the preparation of soaps herein indicated, it may be desirable in some instances to employ as pure rosin acids as possible. These may be prepared from methyl esters of abietic acid or mixtures of rosin acids, which esters are available on the market. This can be accomplished by hydrolyzing the esters in the presence of glycerin with an alkali hydroxide such as potassium hydroxide, dissolving in water, washing with petroleum ether to dissolve out unsaponified materials from the alkali metal soap, adding excess dilute sulfuric acid or other appropriate mineral acid to precipitate out the resultant abietic acid or rosin acid mixture, effecting a solution of resultant rosin acids in petroleum ether or similar light solvent whereby it may be separated from the aqueous solution, recovering the rosin acid solution, removing the light solvent therefrom and then saponifying the resultant rosin acids by methods as heretofore described.

As other sources of abietic acids, I may also use purified or partially purified rosin products such as those known as "commercial abietic acid," "pale wood rosin," such as the grades designated I, K, M, N, WW and WG colors, "FF wood rosin" used in paper sizing, other wood rosins and the

"gum" rosins and corresponding rosin oils. The saponifiable esters present may also be included as acceptable materials; these of course raise the saponification number above the acid or neutralization number. These various rosin materials vary in acid content from about 80% to 90% (calculated as abietic acid) on the average, and from acid numbers of about 150 to about 170 on the average (150 acid number equals about 81% acid and 170 acid number equals about 92% acid).

## BLENDING

For the production of final blends according to the present invention, the concentrates above described are added to lubricating oils of the characters herein defined, preferably at temperatures around 120° F. to 130° F. or 140° F. in proportions to effect the final desired soap content, for example 1.5%, by simple agitation. The concentrate itself may have been prepared with the ordinary California or other ordinary naphthenic base oil containing around 0.5% of sulfur as heretofore described, or with the high sulfur naphthenic base oils heretofore described, or with any suitable blend of the ordinary naphthenic oils and the high sulfur naphthenic oils mentioned, for example to yield from about 1% to almost 3% sulfur as an ordinarily preferable range. Likewise the oil base to which the concentrate is added may consist of one of the ordinary California or other ordinary naphthenic mineral lubricating oils or the high natural sulfur naphthenic base oils or any suitable adjusted blend thereof containing the desired sulfur content.

With respect to the particular high sulfur content naphthenic base oils which are usable, I may mention as appropriate the Santa Maria Valley (California) lubricating oils, the Smack-over (Arkansas) oils, the Spindletop (Texas) oils and certain Mexican oils having the same general characteristics and high sulfur content. These oils after ordinary refining and acid treatment contain ordinarily from about 2.5% sulfur to 4% or 5% sulfur and are therefore very desirable for the present purposes. Similarly shale oils which contain sulfur contents as high as 6% or 7% may also be employed in obtaining suitable blends. Again solvent extract fractions of sulfur-containing petroleum lubricating oils may be employed or added to increase sulfur content. These solvent extracts produced by selective solvent treatment of mineral lubricating oil stocks are well known and possess high sulfur concentration by reason of the removal of the natural sulfur-bearing materials from the stocks. The higher the sulfur content of the stock, the higher the sulfur content of the extract. In general the final sulfur contents of the blended oils vary from about 0.5% sulfur to as high as 4% to 5% sulfur. Where the oils are to be employed with highly corrosion-sensitive alloy bearings, such as cadmium silver bearings, sulfur content preferably should be greater than in the case of Babbitt bearings, and likewise when added oiliness and extreme pressure characteristics are required as is usually the case in Diesel engines and the like, the sulfur content preferably would be higher. Thus, sulfur content may be varied according to requirements. Perhaps it may be stated that in general a sulfur content of around 2% to 3% will meet the greatest number of requirements. This sulfur content, as has already been indicated, acts to overcome corrosive tendencies which may result from hydrolysis of the soaps or may result

from the presence of other corrosive materials added to the blend or to the soap molecule, and also serves to impart added oiliness and extreme pressure characteristics. Such other materials for example, in addition to acids developed by hydrolysis or otherwise, may be represented by chlorine which may be present in the soap molecule by reason of having been introduced into the acid molecule prior to saponification as by chlorination of the rosin acids employed. Again other chlorinated materials may be added to the blend for the purpose of imparting oiliness and extreme pressure characteristics, such as chlorinated methyl ester of abietic acid or chlorinated methyl ester of stearic acid or chloro naphthalene or chlorinated paraffin or chlorinated diphenyl or sulfochlorinated fatty oils or the like.

Typical oils which may be used for producing concentrates and final blends according to the present invention are found in the following California naphthenic base type S. A. E. 30 oil and the Santa Maria Valley naphthenic type S. A. E. 30 lubricating oil.

The California naphthenic S. A. E. 30 oil possesses the following characteristics:

|                                        |         |
|----------------------------------------|---------|
| Gravity A. P. I. at 60° F.             | 20.5    |
| Color N. P. A.                         | 3       |
| Flash C. O. C.                         | 380 30  |
| Fire test C. O. C.                     | 425     |
| Viscosity at 100° F. Saybolt Universal | 571.5   |
| Viscosity at 210° F. Saybolt Universal | 55.3    |
| Pour point                             | -5      |
| Acid number (Method A)                 | 0.04 35 |
| Viscosity index                        | 13      |
| Viscosity gravity constant             | 0.877   |
| Sulfur by weight                       | 0.5%    |
| Indiana oxidation test:                |         |
| Hours for 10 mg. per 10 gm. sample     | 15 40   |
| Hours for 100 mg. per 10 gm. sample    | 35      |
| Ash                                    | Nil     |
| Carbon residue                         | 0.10    |

The Santa Maria Valley S. A. E. 30 naphthenic lubricating oil of the following characteristics was prepared by treatment with 60 pounds of 98% of sulfuric acid per barrel:

|                                            |          |
|--------------------------------------------|----------|
| Gravity A. P. I. at 60° F.                 | 19.0 50  |
| Color N. P. A.                             | 2.4      |
| Flash C. O. C.                             | 390      |
| Fire point C. O. C.                        | 450      |
| Viscosity at 100° F. Saybolt Universal sec | 590 55   |
| Viscosity at 210° F. Saybolt Universal sec | 56       |
| Acid number (Method A)                     | 0.04     |
| Viscosity index                            | 25       |
| Viscosity gravity constant                 | 0.889    |
| Sulfur by weight                           | 3.25% 60 |
| Indiana oxidation test:                    |          |
| Hours for 10 mg. per 10 gm. sample         | 22       |
| Hours for 100 mg. per 10 gm. sample        | 40       |
| Pour point                                 | +15      |

This oil contains natural sulfur content of about 3.25%. Ordinarily a lighter S. A. E. grade thereof will possess a smaller sulfur content, for example about 3%, and a heavier S. A. E. grade ordinarily will have a somewhat greater sulfur content, for example about 3.5%.

An average blend of the two oils of the types above described, in equal quantities possesses the following characteristics, this table covering a blend with and without 1.33% calcium

rosin acid soaps from "commercial abietic acid":

|                                                 | Blend with<br>1.33% calcium<br>abietate | Blend<br>without<br>soap |
|-------------------------------------------------|-----------------------------------------|--------------------------|
| 5 Gravity, A. P. I. at 60° F.                   | 19.2                                    | 19.8                     |
| Viscosity, Saybolt Universal seconds at 100° F. | 732.8                                   | 550                      |
| Viscosity, Saybolt Universal seconds at 210° F. | 58.7                                    | 55                       |
| 10 Viscosity index                              | 0                                       | 15                       |
| Viscosity gravity constant                      | 0.886                                   | 0.884                    |
| Flash, C. O. C. ° F.                            | 370                                     | 370                      |
| Fire, C. O. C. ° F.                             | 435                                     | 445                      |
| Pour point, ° F.                                | 0                                       | +5                       |
| Color, N. P. A.                                 | 44                                      | 3½                       |
| Acid number (mg. KOH/g.)                        | *3.6                                    | **.04                    |
| Sulfated ash, percent by weight                 | 28                                      | NIL                      |
| 15 Sulfur by weight                             | 1.88                                    | 1.88                     |

\*Method B.

\*\*Method A.

Addition agents as herein employed and necessary for these purposes are such as will increase the base oil viscosity only to an inconsequential extent, for example such as indicated in one of the above tables giving data on blends with and without soap. It is to be understood, of course, that a slight viscosity increase such as that imparted by the use of 1.33% of calcium abietate offers no objection.

In addition to using rosin acid soaps of types above indicated, it may also be desirable to sulfurize, or chlorinate, or sulfo-chlorinate such rosin acids and make the soaps therefrom. By sulfurizing, the beneficial effects of sulfur in reducing bearing corrosion may be obtained in the soap, and by chlorinating the increased film strength imparted by chlorine may thereby be obtained in the soap. Both advantages may be obtained by using mixtures of sulfurized and chlorinated materials, or both sulfur and chlorine may be added to the acid molecule as by chlorinating and then sulfurizing, or vice versa, or by treating with a sulfur chloride. For example, sulfurization under mild conditions to effect partial saturation may be followed by chlorination to effect further saturation. The effects of chlorine may be otherwise obtained by using addition agents containing chlorine as hereinbefore indicated, including chlorinated esters such as chlorinated methyl ester of abietic acids, and the valuable effects of sulfur may be otherwise obtained by adding sulfur-bearing materials such as sulfurized oils or fatty oils, organic thio compounds such as organic thiophosphates, sulfurized esters or sulfo-chlorinated esters, such sulfur-bearing methyl ester of abietic or other suitable acids, and the like.

A further use for soaps of abietic acids and other rosin acids is found in their fluidizing properties for grease-like mixtures and other mixtures containing other soaps. For example, a blend of a light Western mineral lubricating oil distillate having a viscosity of 100 seconds Saybolt Universal at 100° F. containing 4% aluminum stearate formed a gel which was reduced to a highly fluid stable oil by the addition of 1% by weight of calcium soaps of tall oil. This suggests the use of calcium abietates in conjunction with other soaps having especially valuable properties in severe service engines where such soaps otherwise tend to separate from the oil or tend inordinately to increase the viscosity of the base oil. I have found, for example, that one-quarter to one-half percent of calcium soaps of commercial abietic acid retains as much as one percent of commercial calcium stearate in stable dispersion or solution in lu-

bricating oils. The present invention however is not intended to extend to those specially treated and modified rosin acid products which have high "grease-setting" or excessive gelling characteristics and therefore would impart excessive viscosity to liquid mineral lubricating oils intended for uses such as internal engine lubrication here described. Such special materials include a rosin product known as "Hyex" as described in the Lister Patent 2,103,204 and British Patent 471,629, and other specially prepared or treated material such as that described in the Brennan et al. Patents 2,042,035 and 2,072,628. On the other hand the materials used in the present invention are predominately unmodified rosin acid compounds and do not substantially increase viscosity in the indicated amounts.

The foregoing disclosures have been furnished for the purpose of indicating preferred and other forms of the invention as they are now understood by applicant, and are to be considered as illustrative and not as limiting.

I claim:

1. A lubricating oil for severe service internal combustion engines comprising a naphthenic base mineral lubricating oil containing between about 1% and 2% of an oil-soluble soap of rosin acids exclusive of those having "high grease-setting properties," the soap having the property of controlling ring sticking in heavy-duty internal combustion engines and free from the property of imparting substantial viscosity increase to the base oil in the stated amounts.

2. A lubricating oil for severe service internal combustion engines comprising mineral naphthenic base lubricating oil containing a stable oil-soluble soap of rosin acids in quantity between about 1% and 3% sufficient to overcome ring sticking and the deposit of gummy, resinous and varnish-like materials in the engine but insufficient to substantially increase the original viscosity of the naphthenic base lubricating oil or impart grease-like characteristics.

3. A lubricating oil according to claim 1 where-  
in the soap is a calcium soap.

4. A lubricating oil according to claim 2 where-  
in the soap is a calcium soap.

5. A lubricating oil for internal combustion engines comprising naphthenic base mineral lub-  
bricating oil naturally containing at least about 0.5% sulfur and an oil-soluble soap of rosin acids in quantity greater than 0.5% but insuffi-  
cient to materially increase the original viscosity of the naphthenic base oil.

6. A lubricating oil for internal combustion engines comprising a sulfur-containing naphthenic base mineral lubricating oil and between about 1% and 2% of an oil-soluble soap of rosin acids, the soap being present in quantity to control ring sticking in heavy-duty internal combustion engines and free from the characteristic of imparting substantial viscosity increase to the base oil in the indicated proportions.

7. A lubricating oil according to claim 1 where-  
in the soap contains at least one of the elements chlorine and sulfur.

8. A lubricating oil for severe service internal combustion engines comprising a mineral lubri-  
cating oil containing between 1% and 2% of an oil-soluble stable soap of rosin acids, the mineral lubricating oil having an acid number of at least about 0.2 by the A. S. T. M. Method B and having good solvent power for the soap, the soap being present in quantity to control ring sticking in

heavy-duty internal combustion engines and free from the characteristic of imparting substantial viscosity increase to the base oil in the indicated proportions.

- 5 9. A lubricating oil for internal combustion engines having non-corrosive characteristics toward alloy bearings highly corrosion-sensitive to organic acidity comprising a naphthenic base mineral lubricating oil having a sulfur content in excess of about 1% and containing between about 0.5% and 3% of an oil-soluble metal soap of rosin acids containing rosin acids imparting an acid number to the oil between about 0.2 and 0.5, the soap being present in quantity sufficient 10 to overcome ring sticking in heavy duty internal combustion engines and insufficient to impart substantial viscosity increase to the base oil.
10. A lubricating oil according to claim 9 wherein the soap is a calcium soap.
- 20 11. A lubricating oil for internal combustion engines of predominantly naphthenic characteristics containing between 0.5% and 3% of oil-soluble soap of rosin acids possessing free acidity, the oil having an acid number between about 0.2 and 0.5 and containing less than about 0.1% 25 water, the soap being present in quantity to control ring sticking in heavy-duty internal combustion engines and free from the characteristic of imparting substantial viscosity increase to the base oil in the indicated proportions.
- 25 12. A mineral lubricating oil for internal combustion engines being free from organic acid corrosion characteristics toward highly corrosion-sensitive alloy bearings and free from grease- 30 like characteristics, comprising a naphthenic base mineral lubricating oil possessing a natural sulfur content in excess of about 1% and containing more than 0.5% of calcium soap of rosin

acids, the oil having an acid number by the A. S. T. M. Method B in excess of about 0.2.

13. A lubricant comprising a naphthenic base mineral lubricating oil naturally having a sulfur content in excess of about 0.5% and a calcium 5 soap of rosin acids, the soap being present in quantity sufficient to overcome ring sticking in heavy duty internal combustion engines and insufficient to impart substantial viscosity increase to the base oil. 10

14. A lubricating oil for heavy duty internal combustion engines comprising a naphthenic base mineral lubricating oil containing between about 0.5% and 3% of a mixture of calcium soaps of rosin acids and calcium soaps of "pine fatty 15 acids."

15. A lubricating oil for heavy service internal combustion engines comprising a naphthenic base mineral lubricating oil containing in excess of about 0.5% sulfur and a mixture of oil-soluble 20 metal soaps of rosin acids and of "pine fatty acids" in amounts in excess of about 0.5% to overcome valve sticking and deposits of resinous and varnish-like materials, and insufficient to materially increase the viscosity of the original 25 naphthenic base oil.

16. A lubricating oil for heavy-duty internal combustion engines comprising mineral lubricating oil containing from about 0.5% to 3% of oil-soluble soap of rosin acids, the soap being present 30 in amount sufficient to overcome ring sticking in an engine but insufficient to increase substantially the original viscosity of the base lubricating oil employed and being free from characteristics of imparting grease-like characteris- 35 tics to the oil in the indicated proportions.

MARCELLUS T. FLAXMAN.